# EUROPEAN PATENT SPECIFICATION

(11) **EP 3 524 707 B1**
(45) Date of publication and mention of the grant of the patent: **07.02.2024**
(21) Application number: 17925535.1
(22) Date of filing: 14.12.2017
(51) Int. Cl.: C22C 38/00, C21D 8/02, C22C 38/60, C22C 38/04, C22C 38/58, C22C 38/02

(54) **STEEL MATERIAL**
STAHLMATERIAL
MATÉRIAU EN ACIER

(43) Date of publication of application: 14.08.2019
(73) Proprietor: Nippon Steel Corporation, Tokyo (JP)
(72) Inventor: SUGAE, Kiyonobu, Chiyoda-ku, Tokyo 100-8071 (JP); DOI, Takashi, Chiyoda-ku, Tokyo 100-8071 (JP); SHIGESATO, Genichi, Chiyoda-ku, Tokyo 100-8071 (JP); KASHIMA, Kazuyuki, Chiyoda-ku, Tokyo 100-8071 (JP)
(74) Representative: Vossius & Partner Patentanwälte Rechtsanwälte mbB
(86) International application number: PCT/JP2017/044984
(87) International publication number: WO 2019/116520

(56) References cited:
- WO-A1-2011/102244
- WO-A1-2011/102244
- WO-A1-2012/133563
- WO-A1-2012/161241
- WO-A1-2014/181534
- JP-A- 2010 007 109
- JP-A- 2012 122 103
- JP-A- 2012 122 103
- JP-A- 2012 255 184
- JP-A- 2014 001 450
- JP-A- 2014 001 450
- JP-B2- 5 958 102
- FUMIMARU K ET AL: "EXTREMELY-LOW CARBON BAINITIC STEELS FOR NEW STRUCTURAL STEEL PRODUCTS", REVUE DE METALLURGIE- CAHIERS D'INFORMATIONS TECHNIQUES,, vol. 97, no. 10, 1 October 2000 (2000-10-01), pages 1235-1244, XP001124153, ISSN: 0035-1563

## Description

### Technical Field

The present disclosure relates to steel material.

### Background Art

In recent years, demand has urgently increased for improvement of the material properties of various steel materials, such as thick steel plates to be used for large structures such as offshore structures built in ice-bound seas, or bridges, and in addition to the improvement of corrosion resistance, there is high demand for the improvement of low-temperature toughness and fatigue characteristics.

Conventionally, an Sn-alloyed steel has been proposed in order to improve corrosion resistance in a seawater environment.

For example, Japanese Patent Application Laid-Open (JP-A) No. 2010-064110, JP-A No. 2012-057236, and JP-A No. 2012-255184 disclose steel materials in which corrosion resistance in an environment containing chloride ions (Cl⁻ ions) is improved by the inclusion of Sn in amounts of from 0.005 to 0.3 mass%, from 0.02 to 0.40 mass%, and from 0.01 to 0.50 mass%, respectively.

Further, JP-A No. 2012-144799 discloses a steel material for an offshore structure containing Sn in amount of from 0.03 to 0.5 mass%, and composed of ferrite and a hard second phase.

Further, Japanese Patent No. 5839151 discloses a technique for improving the corrosion resistance of steel by regulating the Sn concentration ratio between a soft structure and a hard structure by dividing water cooling into two stages.
JP 5958102 relates to a corrosion-resistant steel material for a ship ballast tank which is obtained by heating a steel stock having a composition comprising, by mass, 0.03 to 0.20% C, 0.05 to 0.50% Si, 0.7 to 2.0% Mn, <_0.035% P, <_0.01% S, ≤0.10% Al, 0.02 to 0.2% Sn, 0.003 to 0.03% Nb, 0.005 to 0.030% Ti and 0.0010 to 0.010% N, and in which the contents of Cu, Ni and Cr are controlled to less than 0.20%, less than 0.20% and less than 0.20%, respectively, and the balance Fe with inevitable impurities at 1,000 to 1,350°C, thereafter finishing rolling in the temperature range of 600 to less than 800°C, and performing cooling.
JP 2014-001450 A concerns a steel for ship has a composition that contains, by mass%, C: 0.03 to 0.20%, Si: 0.05 to 0.50%, Mn: 0.7 to 2.00%, Al: 0.100% or less, Ti: 0.005 to 0.030%, N: 0.0010 to 0.010% and Sn: 0.02 to 0.2% and further contains one element or two or more elements selected from Sb: 0.02 to 0.2%, W: 0.005 to 0.50%, Mo: 0.01 to 0.50% and Nb: 0.003 to 0.03%, wherein the remainder of the composition consists of Fe and inevitable impurities, and an area ratio of a ferrite phase is set to 3% or more, and a solid solution amount of Sn after cooling is set to 0.01% or more.
WO 2011/102244 A1 relates to a steel material which has a chemical composition including, by mass%, 0.01-0.14% C, 0.04-0.6% Si, 0.5-2.0% Mn, 0.01% or less P, 0.003% or less S, less than 0.2% Cu, more than 0.0007% but not more than 0.005% B, less than 0.05% Al, less than 0.007% N, 0.003% O, and 0.03-0.50% Sn, with the remainder being Fe and impurities, and the Cu/Sn ratio being 1 or less, and which is characterised in that the Bq value is 0.003 or less, the Ceq value is 0.15-0.35, and the oxide number in the region which is 2 mm or less from the surface layer is 5×10⁴ per 1 square mm.

### SUMMARY OF INVENTION

### Technical Problem

As described above, in order to improve corrosion resistance in a seawater environment or the like, an Sn-alloyed steel has been proposed. However, in addition to improvement of corrosion resistance by the addition of Sn, further improvement of mechanical properties, especially toughness and fatigue characteristics, is required.

For example, with respect to the inventions of JP-A Nos. 2010-064110, 2012-057236, and 2012-255184, which disclose improvement of corrosion resistance by the addition of Sn, there remains room for further improvement in terms of toughness and fatigue characteristics, and a technique that satisfies all of the demands regarding corrosion resistance, toughness, and fatigue characteristics is still required.

In the invention described in JP-A No. 2012-144799, while both corrosion resistance and low-temperature toughness can be improved, there remains room for further improvement with respect to fatigue characteristics.

Further, according to Japanese Patent No. 5839151, the corrosion resistance of steel is improved by regulating the Sn concentration ratio between the soft structure and the hard structure by dividing water cooling into two stages; however, there remains room for further improvement with respect to low-temperature toughness and fatigue characteristics.

An object of the present invention is to provide a steel material which has excellent corrosion resistance as well as low-temperature toughness and fatigue characteristics. Solution to Problem

The present invention was made to achieve the above object with a steel material which is as defined in the claims.

### Advantageous Effects of Invention

According to the present invention it is possible to obtain a steel material with excellent corrosion resistance, low-temperature toughness, and fatigue characteristics.

### DESCRIPTION OF EMBODIMENTS

A steel material according to the present invention will be described in detail.

A numerical range expressed by "from x to y" or "between x and y" includes herein the values of x and y in the range as the minimum and maximum values, respectively.

A steel material according to the invention consists of, in terms of percentage by mass, from 0.01 to 0.20% of C, from 0.01 to 1.00% of Si, from 0.05 to 3.00% of Mn, from 0 to 0.050% of P, from 0 to 0.0100% of S, from 0.05 to 0.25% of Sn, from 0 to 0.100% of Al, from 0.0005 to 0.0100% of N, from 0.0001 to 0.0100% of O, from 0 to 0.050% of Ti, from 0 to 0.050% of Nb, from 0 to 0.050% of V, from 0 to 0.050% of W, from 0 to 0.050% of Mo, from 0 to 0.10% of Cu, from 0 to 0.05% of Ni, from 0 to 0.10% of Cr, from 0 to 0.05% of Sb, from 0 to 0.0010% of B, from 0 to 0.0100% of Ca, from 0 to 0.0100% of Mg, from 0 to 0.0100% of REM, and a balance consisting of Fe and impurities, in which the Sn ratio of the Sn concentration, a, at a crystal grain boundary to the Sn concentration, b, inside a crystal grain, expressed by a/b, is 1.2 or less.

When a steel material of the invention has the above composition, it can be a steel material excellent in corrosion resistance and also in low-temperature toughness and fatigue characteristics. Although the reason therefor is not very clear, it is presumed as follows.

The present inventors prepared various steel plates with different Sn contents, and investigated the relationship between corrosion resistance and toughness. As a result, it has been found that as the Sn content increases, the corrosion resistance improves, but the absorbed energy (low temperature toughness) at 0°C in the Charpy impact test may deteriorate in some cases. For example, when the threshold of corrosion resistance in a SAE J 2334 test is set at 0.6 mm or less, and the threshold of absorbed energy at 0°C is set at 150 J or more, it has been found that not both can be easily satisfied stably.

Therefore, further investigations on corrosion resistance and absorbed energy were conducted, and as a result the composition of steel material, with which excellent absorbed energy could be obtained even at high Sn content, was found.

Further, detailed investigation on the steel material with improved absorbed energy was conducted, and as a result it was found that the ratio between the Sn at the crystal grain boundary and the Sn inside the crystal grain strongly influences the low-temperature toughness of a steel. Also, it was found that the ratio between the Sn at the crystal grain boundary and the Sn inside the crystal grain also influences the fatigue characteristic of a steel. Furthermore, it was found that the same influences the corrosion resistance.

The inventors further studied diligently about a steel material excellent in all of corrosion resistance, low-temperature toughness, and fatigue characteristics, and as a result, the following findings were obtained.

Since the melting point of Sn is low, when Sn is added to a steel material, Sn diffuses within a crystal grain during cooling after rolling and reheating, and segregates at the crystal grain boundary. Then, when Sn segregation at the crystal grain boundary occurs, the toughness of the steel decreases markedly.

In this regard, when segregation of Sn at a crystal grain boundary of Sn in a steel material is suppressed, in particular, when the Sn ratio of the Sn concentration [a] at a crystal grain boundary to the Sn concentration [b] inside a crystal grain, expressed by [a/b] (hereinafter also simply referred to as "the ratio between the Sn at the crystal grain boundary and the Sn inside the crystal grain") is 1.2 or less, it has been found that the low-temperature toughness and the fatigue characteristics are improved, while maintaining excellent corrosion resistance.

The steel material of the present is obtainable by a process including the steps set out in claim 1.

Specifically, a steel after the finish rolling is slowly cooled first, then held at a predetermined temperature for a certain period of time allowing recuperation. Thereafter by conducting strong-cooling to a temperature of 550°C or less, segregation of Sn at a grain boundary can be suppressed, and the Sn ratio can be regulated within the above range.

This invention was devised based on the above findings. Each requirement of the embodiment will be described in detail below.

### (A) Chemical Composition

The reasons for defining the respective elements are as follows. In the following description, "%" for a content means "mass%".

### C: 0.01 to 0.20%

C is an element for improving the strength of a steel material. However, when the C content is excessive, the weldability is remarkably deteriorated. Further, as the C content increases, the formation amount of cementite that acts as a cathode to promote corrosion in a low pH environment increases, and the corrosion resistance of a steel material decreases. Therefore, the C content is defined in a range of from 0.01 to 0.20%. The C content is preferably 0.02% or more, and more preferably 0.03% or more. The lower limit of the C content may be 0.05%, 0.07%, or 0.09%. Further, the C content is preferably 0.18% or less, and more preferably 0.16% or less. The upper limit of the C content may be 0.15%, or 0.13%.

### Si: 0.01 to 1.00%

Si is an element necessary for deoxidation. In order to obtain a sufficient deoxidation effect, it is necessary to contain it 0.01% or more. On the other hand, when the Si content is excessive, the toughness of a steel material, especially when welding is performed, the toughness of a base metal and a weld heat affected zone is impaired. Therefore, the Si content is defined in a range of from 0.01 to 1 .00%. The Si content is preferably 0.03% or more, and more preferably 0.05% or more. The lower limit of the Si content may be 0.10%, 0.15%, or 0.20%. Also, the Si content is preferably 0.80% or less, and more preferably 0.60% or less. The upper limit of the Si content may be 0.50%, 0.40%, or 0.30%.

### Mn: 0.05 to 3.00%

Mn is an element having an action of increasing the strength of a steel material at low cost. However, when the Mn content is excessive, the Mn segregation increases, and the toughness deteriorates. Therefore, the Mn content is defined in a range of from 0.05 to 3.00%. The Mn content is preferably 0.50% or more, and more preferably 0.80% or more. Further, the Mn content is preferably 2.50% or less, and more preferably 2.00% or less.

### P: 0 to 0.050%

P is an element existing as an impurity in a steel material. P is an element that lowers acid resistance of a steel material, and lowers the corrosion resistance of a steel material in a chloride corrosion environment where the pH at a corrosion interface decreases. P also deteriorates the weldability and toughness of a steel material. Therefore, the P content is limited to 0.050% or less. The P content is preferably 0.040% or less, and more preferably 0.030% or less. For improving the toughness, the upper limit of the P content may be 0.020%, 0.015%, or 0.010%. Although it is not easy to completely remove P, it is not necessary to exclude it, and the lower limit of the P content is 0%. Since the desulfurization cost for dephosphorization to ultra-low concentration is high, the lower limit of the P content may be 0.0005%, 0.001%, or 0.003%.

### S: 0 to 0.0100%

S is an element existing as an impurity in a steel material. S forms MnS as a starting point of corrosion in a steel material. When the S content exceeds 0.0100%, the decrease in corrosion resistance of a steel material becomes conspicuous. Therefore, the S content is limited to 0.0100% or less. The S content is preferably 0.0080% or less, more preferably 0.0060% or less, and even more preferably 0.0040% or less. Although it is not easy to remove S completely, it is not necessary to exclude it, and the lower limit of the S content is 0%. Since the refining cost for desulphurization to ultra-low concentration is high, the lower limit of the S content may be 0.0005%, or 0.0010%.

### Sn: 0.05 to 0.25%

Since Sn significantly suppresses an anode dissolution reaction of a steel material in a low pH chloride environment, it greatly improves corrosion resistance of a steel material in a chloride corrosion environment. However, when the Sn content becomes excessive, not only the above effect is saturated, but also the toughness of a steel material, and especially when welding is performed, the toughness of a base material, and a high-heat-input welded joint deteriorates. Therefore, the Sn content is defined in a range of from 0.05 to 0.25%. The Sn content is preferably 0.07% or more, more preferably 0.09% or more, and further preferably 0.10% or more. Further, the Sn content is preferably 0.20% or less, more preferably 0.18% or less, and further preferably 0.016% or less.

### Al: 0 to 0.100%

Al is an element effective for deoxidizing a steel material. Since Si is contained, deoxidation is performed by Si. Therefore, a deoxidation treatment with Al is not absolutely necessary, and the lower limit of the Al content is 0%. However, deoxidation with Al may be performed in addition to the same with Si.
Meanwhile, when the Al content exceeds 0.100%, the corrosion resistance of a steel material in a low pH environment is lowered, so that the corrosion resistance of the steel material in a chloride corrosion environment is lowered. Further, when the Al content exceeds 0.100%, a nitride becomes coarse and the toughness of a steel material decreases. Therefore, the Al content is defined in a range of from 0 to 0.100%. In order to obtain the deoxidation effect with Al, the Al content is preferably 0.005% or more, more preferably 0.010% or more, further preferably 0.015% or more, still further preferably 0.020% or more, and particularly preferably 0.025% or more. Further, the Al content is preferably 0.060% or less, and more preferably 0.045% or less.

### N: 0.0005 to 0.0100%

N dissolves in the form of ammonia and has an effect of improving the corrosion resistance of a steel plate in a saline environment by suppressing the pH decrease due to the hydrolysis of Fe³⁺ in an environment where the amount of air borne salt particle is high. On the other hand, when the N content is excessive, not only the effect is saturated, but also the toughness of a steel plate is deteriorated. Therefore, the N content is regulated in a range of from 0.0005 to 0.0100%. Since it is not easy to lower the lower limit of N below 0.0005%, and it is also costly, the lower limit is set at 0.0005%. The lower limit of the N content may be set at 0.0010% or 0.0020%, according to need. When the content of N exceeds 0.0100%, there arises a risk that coarse AlN is formed and the toughness is apt to decrease, so the upper limit is set at 0.0100%. In order to further increase the toughness, the upper limit of the N content may be set at 0.0080% or 0.0060%.

### O: 0.0001 to 0.0100%

When a steel material contains a trace amount of O (oxygen), the toughness of the same is improved, and especially when welding is applied, the toughness of a welded joint is improved. Meanwhile, O forms an oxide, such as SnO and SnO₂. Therefore, when the O content becomes excessive, when the O content becomes excessive, the Sn concentration in the steel cannot be sufficiently secured. In addition, since the above oxide acts as a starting point of corrosion, the corrosion resistance of a steel material decreases. Therefore, the O content is regulated in a range of from 0.0001 to 0.0100%. The content of O is preferably 0.0002% or more, and more preferably 0.0003% or more. The lower limit of the O content may be 0.0005%, 0.0010%, 0.0015%, or 0.0019%. Also, the O content is preferably 0.0090% or less, and more preferably 0.0080% or less. The upper limit of the O content may be 0.0060%, 0.0040%, or 0.0030%.
Ti: 0 to 0.050%
Nb: 0 to 0.050%
V: 0 to 0.050%

All of Ti, Nb, and V are elements which form precipitates to enhance the strength of a steel material, and may be contained according to need. It is not prerequisite to contain the elements, and the lower limits of their contents are all 0%. On the other hand, when Ti, Nb, or V are excessively contained, the toughness is apt to decrease. Therefore, each content should be 0.050% or less. Each content is preferably 0.0030% or less, and more preferably 0.020% or less. In order to obtain the above effect, one or more kinds selected from Ti, Nb, and V may be contained at 0.001% or more.
W: 0 to 0.050%
Mo: 0 to 0.050%

When the content of W or Mo exceeds 0.050%, the corrosion resistance decreases. Therefore, the contents of W and Mo should be respectively 0.050% or less. It is preferable that both the contents are 0.040% or less. The upper limit of each of the W content and the Mo content may be 0.030%, 0.020%, 0.010%, or 0.005%. In order to improve the corrosion resistance, it is preferable that the W content and the Mo content are as small as possible, and the lower limits of their contents are 0%. However, in order to improve such properties as strength or toughness (especially low-temperature toughness), W and Mo may be contained, and the lower limits of their contents may be 0.010%, or 0.020%.

### Cu: 0 to 0.10%

It is generally believed that Cu is an element that improves the corrosion resistance of a steel material. However, the present inventors have found that the corrosion resistance of a steel material decreases in a corrosive environment containing a chloride as assumed in this embodiment, when it contains Cu. The Cu content is preferably as low as possible, and the lower limit of the Cu content should be 0%. Meanwhile, considering possibility of contamination as an impurity, the Cu content is set at 0.10% or less. For the sake of enhancement of the corrosion resistance, the Cu content is preferably 0.07% or less, more preferably 0.05% or less, further preferably 0.03% or less, and still further preferably 0.02% or less. The Cu content is particularly preferably 0.01% or less.

### Ni: 0 to 0.05%

It is generally believed that Ni improves, similarly to Cu, the corrosion resistance of a steel material. However, the present inventors have found that the corrosion resistance of a steel material decreases in a corrosive environment containing a chloride as assumed in this embodiment, when it contains Ni. The Ni content is preferably as low as possible, and the lower limit of the Ni content should be 0%. Meanwhile, even when it is mixed in as an impurity, so long as the Ni content is 0.05% or less, the corrosion resistance decrease is only slight. Therefore, the Ni content is set at 0.05% or less. For the sake of enhancement of the corrosion resistance, the Ni content is preferably 0.03% or less, more preferably 0.02% or less, and further preferably 0.01% or less.

### Cr: 0 to 0.10%

It is generally believed that Cr is an element that improves corrosion resistance of steel material. However, the present inventors have found that the corrosion resistance of a steel material is deteriorated in a corrosive environment containing a chloride as assumed in this embodiment, when it contains Cr. The Cr content is preferably as low as possible, and the lower limit of the Cr content should be 0%. Meanwhile, considering possibility of contamination as an impurity, the Cr content is set at 0.10% or less. For the sake of enhancement of the corrosion resistance, the Cr content is preferably 0.07% or less, more preferably less than 0.05%, further preferably 0.03% or less, and still further preferably 0.02% or less. The Cr content is particularly preferably 0.01% or less.

### Sb: 0 to 0.05%

Since Sb is an element that improves the acid resistance, Sb may be contained as necessary. It is not indispensable to contain Sb, and the lower limit of its content is 0%. Incidentally, even when Sb is contained in an amount exceeding 0.05%, not only the effect is saturated, but also the toughness and the like of the steel material are deteriorated. Therefore, the Sb content is set at 0.05% or less. The upper limit of the Sb content may be 0.04% or less, or 0.03% or less. In order to obtain the above effect, the Sb content is preferably 0.005% or more, more preferably 0.010% or more, and further preferably 0.015% or more. When it is not necessary to obtain the above effect, the upper limit of the Sb content may be 0.015%, 0.010%, or 0.005% according to need.

### B: 0 to 0.0010%

B is an element for increasing the strength of a steel material by addition of a trace amount thereof, so it may be added optionally. It is not indispensable to contain B, and the lower limit of its content is 0%. When B is added in an amount exceeding 0.0010%, the toughness may be deteriorated, so the B content is set at 0.0010% or less. In order to obtain the above effect, the B content is preferably 0.0003% or more, and more preferably 0.0005% or more. When it is not necessary to obtain the above effect, the upper limit of the B content may be 0.0005%, or 0.0003%, according to need.

### Ca: 0 to 0.0100%

Ca is present in the form of an oxide in a steel material, and has an action of suppressing decrease in pH at the interface in a corrosion reaction zone to prevent corrosion, and therefore Ca may be included if necessary. It is not indispensable to contain Ca, and the lower limit of its content is 0%. When the Ca content exceeds 0.0100%, the above effect is saturated. Accordingly, the Ca content is set at 0.0100% or less. The Ca content is preferably 0.0050% or less, and more preferably 0.0040% or less. In order to obtain the above effect, the Ca content is preferably 0.0002% or more, and more preferably 0.0005% or more. When it is not necessary to obtain the above effect, the upper limit of the Ca content may be 0.0030%, 0.0005%, or 0.0002% or less, according to need.

### Mg: 0 to 0.0100%

Similar to Ca, Mg has an action of suppressing decrease in pH at the interface in a corrosion reaction zone to prevent corrosion of a steel material, and therefore Mg may be included according to need. It is not indispensable to contain Mg, and the lower limit of its content is 0%. When the Mg content exceeds 0.0100%, the above effect is saturated. Therefore, the Mg content is set at 0.0100% or less. The Mg content is preferably 0.0050% or less, and more preferably 0.0040% or less. In order to obtain the above effect, the Mg content is preferably 0.0002% or more, and more preferably 0.0005% or more. When it is not necessary to obtain the above effect, the upper limit of the Mg content may be set at 0.0030%, 0.0005%, or 0.0002%, according to need.

### REM: 0 to 0.0100%

Since REM (rare earth element) is an element that improves the weldability of a steel material, it may be included as necessary. It is not indispensable to contain REM, and the lower limit of its content is 0%. When the REM content exceeds 0.0100%, the above effect is saturated. Therefore, the REM content should be 0.0100% or less. The REM content is preferably 0.0050% or less, and more preferably 0.0040% or less. In order to obtain the above effect, the REM content is preferably 0.0002% or more, and more preferably 0.0005% or more. When it is not necessary to obtain the above effect, the upper limit of the Mg content may be set at 0.0030%, 0.0005%, or 0.0002%, according to need.

In this regard, REM is a collective term of 17 elements including 15 elements of lanthanoid, as well as Y and Sc. One or more of these 17 elements may be included in a steel material, and the REM content means the sum of the contents of such elements.

The balance of the chemical composition is Fe and impurities.

In this regard, "impurity" means a component which is mixed in when a steel material is produced industrially due to various factors related to the raw material, such as ore, and scrap, or a production process, and which is tolerable so long as the invention is not adversely affected.

### (B) Sn Ratio

The Sn ratio of the Sn concentration [a] at a crystal grain boundary to the Sn concentration [b] inside a crystal grain, expressed by [a/b]: 1.2 or less

As described above, the Sn ratio between the crystal grain boundary and the crystal grain inside affects the low-temperature toughness, the fatigue characteristics and the corrosion resistance of a steel. When Sn is segregated at the crystal grain boundary and the Sn ratio between the crystal grain boundary and the crystal grain inside exceeds 1.2, the improvement effect on the low-temperature toughness and the fatigue characteristics cannot be expected. Therefore, the Sn ratio between the crystal grain boundary and the crystal grain inside is set at 1.2 or less. The Sn ratio is preferably 1.1 or less, and more preferably 1.05 or less. Although the lower limit of the Sn ratio need not be particularly determined, the lower limit may be set at 0.7, 0.8, 0.9, or 1.0.

There is no precipitate of Sn in a steel material of the invention and the extraction residue is 0%. That is, all of Sn is dissolved as a solid solution in a steel material.

An Sn ratio between the crystal grain boundary and the crystal grain inside of the invention may be determined by the following method. Firstly, a cylindrical specimen having a diameter of 3 mm and a length of 10 mm is prepared from a steel material at a position of 1/4 t (t represents plate thickness or wall thickness). Then, the specimen was subjected to an ultra-high vacuum impact fracture mechanism attached to an Auger spectroscopic analyzer (Model 670i, manufactured by ULVAC-PHI, Inc.), and the fracture surface, which is formed by fracture in vacuum (1.0E⁻⁹ Torr or less) in an atmosphere at the liquid nitrogen temperature (-150°C), is observed. The fracture surface is mostly occupied by cleavage fracture surfaces having a river pattern, and dimple fracture surfaces, and sparse intergranular fractured surfaces are also recognized. The crystal grain boundary and the crystal grain inside of the fracture surface are discriminated by a macro-fractographic method, and Auger spectra are measured at 10 positions in each crystal grain boundary and crystal grain inside. To verify the discrimination between the crystal grain boundary and the crystal grain inside, the fracture surface examined by the macro-fractographic method is analyzed by Auger spectroscopy with respect to C, which is apt to segregate at a crystal grain boundary, to confirm discrimination between the crystal grain boundary and the crystal grain inside. The Sn ratio is calculated by measuring the ratio of the concentrations (atom%) of Sn between the crystal grain boundary and the crystal grain inside. In this regard, the relative sensitivity coefficient is calibrated with Au.

### (C) Dimensions

There is no particular restriction on the dimensions such as the thickness of a steel material of the invention.

However, the effect of improving the corrosion resistance, the low-temperature toughness, and the fatigue resistance is more remarkably obtained when a steel material is used in a form of a steel plate having a thickness of from 6 to 100 mm. The thickness (plate thickness) of a steel plate is preferably from 10 to 40 mm. A steel material may be a steel pipe or a section steel, and its thickness or wall thickness may be from about 3 to 50 mm.

### (D) Production Method

A steel material according to the invention can be produced using, for example, the production method described below.

Namely a method of producing a steel material including:
a step of preparing a slab whose chemical composition is the same as the above composition,
a heating step of heating the slab to a temperature in the range of from 1000 to 1150°C,
a rough rolling step of applying rough rolling to the slab,
a finish rolling step of applying finish rolling to the slab having undergone rough rolling to provide a finishing temperature of the surface of from 900 to 750°C and a
   rolling reduction rate from 950°C of 50% or higher,
a first accelerated cooling step of performing accelerated cooling of the finish-rolled slab (steel material) at a cooling rate of from 5 to 10°C/s until the surface temperature reaches 630°C or less,
a recuperation step of suspending accelerated cooling of the slab (steel material) after the first accelerated cooling step and allowing cooling in the air for 30 to 120 sec (suspension of accelerated cooling and cooling in the air is hereinafter referred to as "holding"), and further allowing recuperation by the heat from the inside of the slab (steel material) until the surface temperature reaches a range of from 650 to 700°C
a second accelerated cooling step of performing accelerated cooling of the slab (steel material) after the recuperation step at a cooling rate of from 10 to 60°C/s until the surface temperature reaches 550°C or less, and
an air cooling step of performing cooling in the air after the second accelerated cooling step.

The heating temperature in the heating step is from 1000 to 1150°C. When the temperature is within the above range, the austenite grain size at the time of heating can be kept small, so that grain refining of the rolled structure can be achieved. When the heating temperature is 1150°C or lower, coarsening of austenite grains is suppressed and coarsening of the structure after cooling transformation is also suppressed, so that excellent low-temperature toughness can be achieved. On the other hand, when the heating temperature is 1000°C or higher, the alloy elements are sufficiently solutionized, so that the deterioration of the internal quality of the steel is suppressed, and the finishing temperature in rolling is not excessively lowered, so that the enhancement of low-temperature toughness can be expected.

Further, when the finishing temperature at the surface in the rolling step is 900°C or lower, the growth of recrystallized austenite grains is suppressed, and grain refining thereof is promoted. Further, when the finishing temperature is 750°C or higher, the ferrite structure becomes less susceptible to processing, so that the low-temperature toughness is improved. Consequently, the finishing temperature is set from 900 to 750°C.

Furthermore, when the rolling reduction rate from 950°C is 50% or more, partial recrystallization of austenite hardly occurs, so that a duplex grain structure is suppressed to enhance the low-temperature toughness. Consequently, the rolling reduction rate from 950°C is set at 50% or more.

Regarding cooling after rolling, water cooling is carried out under the following conditions.

### <Slow Cooling After Completion of Rolling (First Accelerated Cooling Step)>

After finish rolling, accelerated cooling is immediately performed at a cooling rate of from 5 to 10°C/s until the surface temperature of a steel material becomes 630°C or lower. With the cooling rate within the above range, grain boundary segregation of Sn can be suppressed. When the cooling rate is 5°C/s or more, Sn diffusion is suppressed. When it is 10°C/s or less, the Sn ratio between the crystal grain boundary and the crystal grain inside is reduced, although the reason therefor is not very clear. As a result, in both cases, the low-temperature toughness and the fatigue characteristics are improved.

### <Recuperation by Holding before Accelerated Cooling (Recuperation Step)>

After slow cooling, the accelerated cooling is suspended allowing cooling in the air (holding) for recuperation until the surface temperature of the cooled steel material rises again due to the internal temperature of the steel material and the surface temperature is equalized in a temperature range of from 650 to 700°C. The holding time (this time is the accelerated cooling suspension time corresponding to the recuperation time) is 30 to 120 sec. Owing to the recuperation step, it is possible to segregate elements that are apt to segregate, such as S, P, and C, into the crystal grain boundary, and to suppress diffusion of Sn. When the holding time is 30 sec or more, uniform recuperation deep into the inside of a steel material becomes possible. When the holding time is 120 seconds or less, elevation of the surface temperature of a steel material up to a temperature range exceeding 700°C may be suppressed more easily so that diffusion of Sn may be reduced to suppress segregation.

### <Accelerated Cooling (Second Accelerated Cooling Step)>

Thereafter, cooling is resumed at a cooling rate of from 10 to 60°C/s until the surface temperature reaches 550°C or less. By accelerated cooling under the above conditions, it is possible to suppress segregation of Sn at the crystal grain boundary, and to refine the steel structure. When the cooling rate is 10°C/s or more, diffusion of Sn is suppressed, and segregation at the grain boundary is suppressed. Meanwhile, when the cooling rate is 60°C/s or less, an increase in the strength of a steel material plate is suppressed, and the fatigue resistance is improved.

After the second accelerated cooling step, cooling in the air is performed. In a case where a steel material of the invention is used for a large structure, such as a bridge and an offshore structure, the tensile strength should preferably be in a range of from 400 to 650 MPa. The tensile strength may be also from 480 to 580 MPa.

### EXAMPLES

The present invention will be described more specifically below by way of Examples, provided that the present disclosure is not limited to the Examples.

A steel having the chemical composition shown in Table 1 was melted in a furnace and then cast in to a slab with a thickness of 300 mm. The slab was heated, subjected to rough rolling and finish rolling, and then quickly cooled to a steel plate having a plate thickness of 20 mm. The production conditions are shown in Table 2.

**[Table 1]**

| Steel grade | Chemical composition (mass%, balance: Fe and impurities) | | | | | | | | | | |
|---|---|---|---|---|---|---|---|---|---|---|---|
| | C | Si | Mn | P | S | Sn | Al | N | O | Ti | Nb |
| A | 0.13 | 0.33 | 1.41 | 0.010 | 0.0030 | 0.18 | 0.033 | 0.0041 | 0.0050 | | |
| B | 0.12 | 0.31 | 1.33 | 0.001 | 0.0010 | 0.12 | 0.020 | 0.0028 | 0.0010 | | |
| C | 0.10 | 0.31 | 1.30 | 0.003 | 0.0100 | 0.11 | 0.040 | 0.0038 | 0.0030 | | |
| D | 0.14 | 0.36 | 1.22 | 0.010 | 0.0080 | 0.09 | 0.027 | 0.0024 | 0.0030 | | |
| E | 0.11 | 0.34 | 1.13 | 0.050 | 0.0050 | 0.20 | 0.036 | 0.0033 | 0.0050 | | |
| F | 0.12 | 0.38 | 1.62 | 0.005 | 0.0010 | 0.17 | 0.023 | 0.0020 | 0.0002 | 0.011 | 0.024 |
| G | 0.13 | 0.31 | 1.13 | 0.003 | 0.0060 | 0.09 | 0.023 | 0.0036 | 0.0080 | | |
| H | 0.08 | 0.21 | 1.90 | 0.010 | 0.0005 | 0.12 | 0.025 | 0.0045 | 0.0050 | | |
| I | 0.08 | 0.28 | 1.02 | 0.005 | 0.0030 | 0.19 | 0.031 | 0.0034 | 0.0050 | | 0.016 |
| J | 0.12 | 0.21 | 1.94 | 0.001 | 0.0010 | 0.05 | 0.023 | 0.0026 | 0.0030 | 0.015 | 0.008 |
| K* | 0.08 | 0.21 | 1.02 | 0.003 | 0.0030 | 0.05 | 0.020 | 0.0030 | 0.0020 | | |
| L* | 0.13 | 0.31 | 1.13 | 0.005 | 0.0010 | 0.12 | 0.020 | 0.0030 | 0.0030 | | |
| M* | 0.08 | 0.28 | 1.02 | 0.050 | 0.0050 | 0.19 | 0.031 | 0.0034 | 0.0050 | | |
| N* | 0.10 | 0.25 | 1.13 | 0.003 | 0.0050 | 0.12 | 0.030 | 0.0020 | 0.0030 | | |
| O* | 0.13 | 0.32 | 1.25 | 0.005 | 0.0050 | - | 0.030 | 0.0036 | 0.0030 | | |
| P* | 0.10 | 0.22 | 1.17 | 0.010 | 0.0030 | 0.02 | 0.030 | 0.0040 | 0.0030 | | |
| Q* | 0.14 | 0.25 | 1.61 | 0.005 | 0.0080 | 0.30 | 0.028 | 0.0034 | 0.0050 | | |
| | | | | | | | | | | | |

| | V | W | Mo | Cu | Ni | Cr | Sb | B | Ca | Mg | REM |
|---|---|---|---|---|---|---|---|---|---|---|---|
| A | | | 0.030 | | 0.01 | | | | | | |
| B | | | | | | | | | | | |
| C | | | | | 0.01 | | | | | | |
| D | | | | | | | | | | | |
| E | | | 0.020 | | | | | | | | |
| F | | 0.011 | | 0.07 | 0.03 | | | 0.0003 | | | |
| G | 0.009 | | | | | | | | 0.0004 | | |
| H | | | 0.010 | | | | | 0.0002 | | 0.0033 | |
| I | | | | | | 0.01 | | | | | 0.0019 |
| J | 0.007 | | | 0.03 | | | 0.01 | | | | |
| K | | | | 0.12 | | | | | | | |
| L | | | 0.070 | | 0.02 | | | | | | |
| M | | | | | 0.07 | | | | | | |
| N | | | | | | 1.10 | | | | | |
| O | | | 0.030 | | 0.03 | | | | | | |
| P | | | 0.010 | | | | | | | | |
| Q | | | | | 0.01 | | | | | | |

| | | | | | | | | | | | |
|---|---|---|---|---|---|---|---|---|---|---|---|
| Steel compositions not fulfilling the requirements of claim 1 are marked with an asterisk (*) | | | | | | | | | | | |

**[Table 2]**

| Test No. | Steel grade | Rolling step | | | 1st accelerated cooling step | | Recuperation step | | 2nd accelerated cooling step | |
|---|---|---|---|---|---|---|---|---|---|---|
| | | Heating temperature (°C) | Finishing temperature (°C) | Reduction rate from 950°C | Slow cooling rate (°C/s) | Cooling completion temperature (°C) | Holding time (s) | Holding time completion temperature (°C) | Accelerated cooling rate (°C/s) | Cooling completion temperature (°C) |
| 1 | A | 1150 | 850 | 52 | 7 | 600 | 60 | 680 | 30 | 500 |
| 2 | B | 1150 | 800 | 55 | 6 | 580 | 30 | 650 | 10 | 520 |
| 3 | C | 1120 | 750 | 55 | 7 | 620 | 30 | 650 | 40 | 450 |
| 4 | D | 1150 | 840 | 50 | 7 | 600 | 60 | 660 | 50 | 400 |
| 5 | E | 1120 | 890 | 52 | 6 | 630 | 90 | 700 | 20 | 520 |
| 6 | F | 1150 | 900 | 55 | 5 | 580 | 120 | 700 | 20 | 500 |
| 7 | G | 1000 | 810 | 58 | 10 | 600 | 60 | 650 | 20 | 550 |
| 8 | H | 1150 | 880 | 55 | 6 | 600 | 60 | 690 | 40 | 500 |
| 9 | I | 1150 | 750 | 55 | 7 | 620 | 30 | 660 | 20 | 520 |
| 10 | J | 1120 | 860 | 50 | 5 | 630 | 30 | 670 | 30 | 480 |
| 11 | K | 1150 | 860 | 52 | 6 | 600 | 60 | 660 | 30 | 450 |
| 12 | L | 1120 | 860 | 55 | 5 | 600 | 30 | 660 | 20 | 400 |
| 13 | M | 1150 | 890 | 50 | 7 | 580 | 60 | 700 | 40 | 520 |
| 14 | N | 1150 | 890 | 55 | 6 | 620 | 90 | 700 | 30 | 500 |
| 15 | O | 1120 | 890 | 55 | 6 | 620 | 60 | 700 | 30 | 520 |
| 16 | P | 1120 | 850 | 55 | 5 | 600 | 60 | 680 | 30 | 500 |
| 17 | Q | 1120 | 850 | 52 | 5 | 580 | 60 | 650 | 30 | 520 |
| 18 | A | 1150 | 850 | 50 | 2 | 650 | 90 | 680 | 30 | 500 |
| 19 | A | 1150 | 850 | 50 | 30 | 520 | 30 | 600 | 30 | 520 |
| 20 | A | 1150 | 850 | 50 | 6 | 600 | 120 | 720 | 30 | 520 |
| 21 | A | 1150 | 850 | 55 | 6 | 620 | 0 | - | 30 | 500 |
| 22 | A | 1150 | 850 | 50 | 10 | 600 | 30 | 650 | 8 | 560 |
| 23 | A | 1150 | 850 | 50 | 6 | 620 | 30 | 650 | 65 | 380 |

| | | | | | | | | | | |
|---|---|---|---|---|---|---|---|---|---|---|
| Test Nos. 11 to 23 do not fulfill the requirements of claim 1 | | | | | | | | | | |

Subsequently, a cylindrical specimen having a diameter of 3 mm and a length of 10 mm was cut out from each steel plate, and subjected to an ultra-high vacuum impact fracture mechanism attached to an Auger spectroscopic analyzer (Model 670i, manufactured by Ulvac Inc.), and the fracture surface, which was formed by fracture in vacuum (1.0E-9 Torr or less) in an atmosphere at the liquid nitrogen temperature (-150°C), was observed. The fracture surface was mostly occupied by cleavage fracture surfaces having a river pattern, and dimple fracture surfaces, and sparse intergranular fractured surfaces were also recognized. The crystal grain boundary and the crystal grain inside of the fracture surface were discriminated by a macro-fractographic method, and Auger spectra were measured at 10 positions in each crystal grain boundary and crystal grain inside. To verify the discrimination between the crystal grain boundary and the crystal grain inside, the fracture surface examined by the macro-fractographic method was analyzed by Auger spectroscopy with respect to C, which was apt to segregate at a crystal grain boundary, to confirm discrimination between the crystal grain boundary and the crystal grain inside. The Sn ratio was calculated by measuring the ratio of the concentrations (atom%) of Sn between the crystal grain boundary and the crystal grain inside. In this regard, the relative sensitivity coefficient was calibrated with Au.

Further, a corrosion resistance test, a toughness test, and a fatigue test were conducted for each steel plate.

### <Corrosion Resistance Test>

A specimen having a length of 60 mm, a width of 100 mm, and a thickness of 3 mm was cut out from each steel plate, and subjected to the SAE J 2334 test. In doing so, two specimens were taken from each steel plate, and on one of them, an anticorrosion coating was formed in advance. The SAE J 2334 test will be described below.

The SAE J 2334 test is an accelerated deterioration test in which a cycle of humid stage and dry stage (humid → salt application → dry; 24 hours in total) is repeated to simulate a severely corrosive environment where the amount of air borne salt particle exceeds 1 mdd. The SAE J 2334 test was conducted repeating a cycle under the following conditions. The corrosion form under the following conditions is similar to the corrosion form of an atmospheric exposure test.

### (Test Conditions)

Humid stage: 50°C, 100% RH, 6 hours,
Salt application stage: Immersion in the aqueous solution with 0.5 mass% of NaCl, 0.1 mass% of CaCl₂, and 0.075 mass% of NaHCO₃ for 0.25 hours,
Dry stage: 60°C, 50% RH, 17.75 hours.

In addition, a shotblasting treatment was applied to the surface of each specimen. With respect to some specimens, after the shotblasting treatment, an anticorrosion primary coating, an under coating, an intermediate coating, and an over coating were applied one on another to form an anticorrosion coating having a total thickness of 250 µm.

As the anticorrosion primary coating, an inorganic zinc rich paint ("SHINTO-ZINC #2000" produced by SHINTO PAINT CO., LTD.) was coated to a thickness of 75 µm, and as a mist coating an epoxy resin paint ("NEO-GOSE #2300 MC" produced by SHINTO PAINT CO., LTD.) was applied. As the under coating, an epoxy resin coating ("NEO-GOSE #2300 PS" produced by Shinto Paint Co., Ltd.) was spray-coated to a film thickness of 120 µm. In addition, as the intermediate coating, an intermediate paint for a fluorine resin paint ("SHINTO-FLON #100 intermediate paint" produced by SHINTO PAINT CO., LTD.) was coated to a thickness of 30 µm. Further, as the over coating, a fluorine resin coating ("SHINTO-FLON #100" produced by SHINTO PAINT CO., LTD.) was spray-coated to a film thickness of 25 µm.

For each specimen having the anticorrosion coating, a cross scratch was formed on the anticorrosion coating to expose part of the steel material. With respect to each of the specimens on which an anticorrosion coating was not formed, rust was formed uniformly over the entire specimen surface after the test, and therefore its corrosion amount was determined. The "corrosion amount" was determined as the average plate thickness decrement of the specimen when a surface rust layer on the surface was removed. Specifically, the plate thickness decrement was calculated using the weight change of the specimen before and after the test, and the surface area of the specimen, and used as the corrosion amount.

The criteria for pass or fail at a corrosion resistance test were as follows. A SAE J 2334 test was conducted for 120 cycles using a specimen on which an anticorrosion coating was not formed, and one in which the corrosion amount was 0.60 mm or less was judged for passed. Further, a SAE J2334 test was conducted for 200 cycles using a specimen on which an anticorrosion coating was formed, and one in which the detached area at a scratched zone was 20% or less, and the maximum corrosion depth was 0.40 mm or less was judged as pass.

### <Low-temperature Toughness Test>

The low-temperature toughness was evaluated on an impact test specimen taken from a central part in the plate thickness direction of the plate and in the direction perpendicular to the rolling direction, by determining the absorbed energy (vE₀) at 0°C using a V-notch specimen according to JIS Z 2242. A specimen with an absorbed energy of 150 J or more was judged as pass.

### <Fatigue Test>

In a fatigue test, the stress amplitude was changed as a test parameter, and the relationship between the stress amplitude and the fatigue fracture life was represented by a S-N diagram, and a fatigue limit was derived therefrom. In the fatigue test, a No. 2 specimen specified in JIS Z 2275 was used, and the load ratio (the value obtained by dividing the minimum load by the maximum load) was set at 0.1. In this regard, the fatigue fracture life was defined as the time point at which the displacement (the displacement of the cylinder of an actuator that applied the load to a specimen) at the maximum load increased by 1 mm as compared with the start of the test. When the fatigue fracture life was 5.5×10⁵ cycles or more, the fatigue resistance was judged as pass.

The results are summarized in Table 3.

**[Table 3]**

| Test No. | Steel grade | Sn ratio between grain boundary and grain inside | SAE 12334 test without a coating 120CY | SAE J2334 test with a coating 200CY | | Absorbed energy (J) | Fatigue characteristics (×10⁵) | |
|---|---|---|---|---|---|---|---|---|
| | | | Corrosion amount (mm) | Detached area (%) | Maximum corrosion depth (mm) | | | |
| 1 | A | 1.1 | 0.50 | 20 | 0.38 | 150 | 6.2 | Example of present disclosure |
| 2 | B | 1.1 | 0.40 | 15 | 0.35 | 155 | 6.0 | |
| 3 | C | 1.1 | 0.50 | 20 | 0.35 | 162 | 6.2 | |
| 4 | D | 1.2 | 0.60 | 20 | 0.30 | 150 | 6.5 | |
| 5 | E | 1.1 | 0.50 | 20 | 0.38 | 158 | 6.0 | |
| 6 | F | 1.1 | 0.50 | 20 | 0.38 | 155 | 6.7 | |
| 7 | G | 1.2 | 0.60 | 20 | 0.35 | 150 | 6.0 | |
| 8 | H | 1.0 | 0.40 | 15 | 0.35 | 155 | 6.8 | |
| 9 | I | 1.1 | 0.60 | 15 | 0.30 | 162 | 6.0 | |
| 10 | J | 1.2 | 0.50 | 20 | 0.35 | 155 | 6.5 | |
| 11 | K | 1.1 | 0.70 | 50 | 0.45 | 140 | 5.5 | Comparative Example |
| 12 | L | 1.0 | 0.80 | 45 | 0.50 | 150 | 6.5 | |
| 13 | M | 1.1 | 1.10 | 55 | 1.20 | 155 | 6.0 | |
| 14 | N | 1.1 | 1.50 | 60 | 1.60 | 165 | 6.0 | |
| 15 | O | - | 1.50 | 50 | 1.10 | 165 | 6.0 | |
| 16 | P | 0.7 | 1.15 | 20 | 0.30 | 145 | 5.5 | |
| 17 | Q | 1.3 | 0.40 | 25 | 0.30 | 143 | 5.8 | |
| 18 | A | 1.7 | 0.70 | 35 | 0.45 | 146 | 3.9 | |
| 19 | A | 1.8 | 0.70 | 30 | 0.40 | 145 | 5.8 | |
| 20 | A | 1.5 | 0.80 | 30 | 0.42 | 148 | 3.7 | |
| 21 | A | 1.6 | 0.70 | 25 | 0.45 | 146 | 4.3 | |
| 22 | A | 1.6 | 0.70 | 20 | 0.42 | 145 | 5.5 | |
| 23 | A | 1.5 | 0.70 | 30 | 0.45 | 143 | 4.5 | |

Test Nos. 1 to 10 are Examples of the present disclosure which satisfy all the requirements of the present disclosure. As obvious from Table 3, in the SAE J 2334 test, the corrosion amount of the specimen without a coating was 0.60 mm or less, and in the scratched zone of the specimen with a coating the detached area was 20% or less, and the maximum corrosion depth was 0.40 mm or less. In the toughness test, the Charpy absorbed energy at 0°C was 150 J or more. Further, in the fatigue test, the fatigue fracture life was 5.5 × 10⁵ cycles or more.

In contrast thereto, in Test Nos. 15 and 16, which were Comparative Examples, the Sn content in the steel material was less than the defined lower limit value, and consequently the corrosion resistance was inferior. Further, in Test No. 17, in which the Sn content in the steel material exceeded the defined upper limit value, the Sn ratio between the crystal grain boundary and the crystal grain inside exceeded 1.2, and as a result the low-temperature toughness and the fatigue resistance were inferior.

Further, in Test Nos. 18 to 23, the Sn ratio between the crystal grain boundary and the crystal grain inside exceeded 1.2, and as a result the corrosion resistance slightly decreased, and the low-temperature toughness and the fatigue resistance were also inferior.

Further, in Test Nos. 11 to 14, which were Comparative Examples, the content of Mo, Cu, Ni, or Cr in the steel material exceeded the defined upper limit value, and as a result the corrosion resistance was inferior.

### INDUSTRIAL APPLICABILITY

According to the present invention it becomes possible to obtain a steel material excellent in corrosion resistance, low-temperature toughness, and fatigue characteristics. Therefore, a steel material according to the present disclosure is suitable for use as a material for a large structure, such as an offshore structure used in a cold district, and a bridge.

## Claims

1. A steel material, consisting of in terms of percentage by mass:
from 0.01 to 0.20% of C,
from 0.01 to 1.00% of Si,
from 0.05 to 3.00% of Mn,
from 0 to 0.050% of P,
from 0 to 0.0100% of S,
from 0.05 to 0.25% of Sn,
from 0 to 0.100% of Al,
from 0.0005 to 0.0100% of N,
from 0.0001 to 0.0100% of O,
from 0 to 0.050% of Ti,
from 0 to 0.050% of Nb,
from 0 to 0.050% of V,
from 0 to 0.050% of W,
from 0 to 0.050% of Mo,
from 0 to 0.10% of Cu,
from 0 to 0.05% of Ni,
from 0 to 0.10% of Cr,
from 0 to 0.05% of Sb,
from 0 to 0.0010% of B,
from 0 to 0.0100% of Ca,
from 0 to 0.0100% of Mg,
from 0 to 0.0100% of REM, and
a balance consisting of Fe and impurities,
wherein an Sn ratio of an Sn concentration, a in atom%, at a crystal grain boundary to an Sn concentration, b in atom%, inside a crystal grain, expressed by a/b, is 1.2 or less, determined by a measuring method as described in the section "(B) Sn Ratio" of the description wherein the steel material is obtainable by a method containing the following steps:
a step of preparing a slab having a chemical composition as indicated above with respect to the steel material,
a heating step of heating the slab to a temperature in the range of from 1000 to 1150°C,
a rough rolling step of applying rough rolling to the slab,
a finish rolling step of applying finish rolling to the slab having undergone rough rolling to provide a finishing temperature of the surface of from 900 to 750°C and a rolling reduction rate from 950°C of 50% or higher,
a first accelerated cooling step of performing accelerated cooling of the finish-rolled steel material at a cooling rate of from 5 to 10°C/s until the surface temperature reaches 630°C or less,
a recuperation step of suspending accelerated cooling of the steel material after the first accelerated cooling step and allowing cooling in the air for 30 to 120 sec, and further allowing recuperation by the heat from the inside of the steel material until the surface temperature reaches a range of from 650 to 700°C,
a second accelerated cooling step of performing accelerated cooling of the steel material after the recuperation step at a cooling rate of from 10 to 60°C/s until the surface temperature reaches 550°C or less, and
an air cooling step of performing cooling in the air after the second accelerated cooling step.

2. The steel material according to claim 1 in a form of steel plate with a plate thickness of from 6 to 100 mm.

3. A method of producing a steel material, wherein the method includes:
a step of preparing a slab consisting of in terms of percentage by mass:
from 0.01 to 0.20% of C,
from 0.01 to 1.00% of Si,
from 0.05 to 3.00% of Mn,
from 0 to 0.050% of P,
from 0 to 0.0100% of S,
from 0.05 to 0.25% of Sn,
from 0 to 0.100% of Al,
from 0.0005 to 0.0100% of N,
from 0.0001 to 0.0100% of O,
from 0 to 0.050% of Ti,
from 0 to 0.050% of Nb,
from 0 to 0.050% of V,
from 0 to 0.050% of W,
from 0 to 0.050% of Mo,
from 0 to 0.10% of Cu,
from 0 to 0.05% of Ni,
from 0 to 0.10% of Cr,
from 0 to 0.05% of Sb,
from 0 to 0.0010% of B,
from 0 to 0.0100% of Ca,
from 0 to 0.0100% of Mg,
from 0 to 0.0100% of REM, and
a balance consisting of Fe and impurities,
a heating step of heating the slab to a temperature in the range of from 1000 to 1150°C,
a rough rolling step of applying rough rolling to the slab,
a finish rolling step of applying finish rolling to the slab having undergone rough rolling to provide a finishing temperature of the surface of from 900 to 750°C and a rolling reduction rate from 950°C of 50% or higher,
a first accelerated cooling step of performing accelerated cooling of the finish-rolled steel material at a cooling rate of from 5 to 10°C/s until the surface temperature reaches 630°C or less,
a recuperation step of suspending accelerated cooling of the steel material after the first accelerated cooling step and allowing cooling in the air for 30 to 120 sec, and
further allowing recuperation by the heat from the inside of the steel material until the surface temperature reaches a range of from 650 to 700°C,
a second accelerated cooling step of performing accelerated cooling of the steel material after the recuperation step at a cooling rate of from 10 to 60°C/s until the surface temperature reaches 550°C or less, and
an air cooling step of performing cooling in the air after the second accelerated cooling step;
to provide a steel material having an Sn ratio of an Sn concentration, a in atom%, at a crystal grain boundary to an Sn concentration, b in atom%, inside a crystal grain,
expressed by a/b, is 1.2 or less, determined by a measuring method as described in the section "(B) Sn Ratio" of the description.

4. The method according to claim 3, wherein the steel material is in a form of steel plate with a plate thickness of from 6 to 100 mm.

## Patentansprüche

1. Ein Stahlmaterial, bestehend aus, in Massenprozent:
von 0,01 bis 0,20% C,
von 0,01 bis 1,00% Si,
von 0,05 bis 3,00% Mn,
von 0 bis 0,050% P,
von 0 bis 0,0100% S,
von 0,05 bis 0,25% Sn,
von 0 bis 0,100% Al,
von 0,0005 bis 0,0100% N,
von 0,0001 bis 0,0100% O,
von 0 bis 0,050% Ti,
von 0 bis 0,050% Nb,
von 0 bis 0,050% V,
von 0 bis 0,050% W,
von 0 bis 0,050% Mo,
von 0 bis 0,10% Cu,
von 0 bis 0,05% Ni,
von 0 bis 0,10% Cr,
von 0 bis 0,05% Sb,
von 0 bis 0,0010% B,
von 0 bis 0,0100% Ca,
von 0 bis 0,0100% Mg,
von 0 bis 0,0100% Seltenerdmetallen und
einem Rest, der aus Fe und Verunreinigungen besteht,
wobei ein Sn-Verhältnis einer Sn-Konzentration, a, in Atom-%, an einer Kristallkorngrenze zu einer Sn-Konzentration, b, in Atom-%, im Inneren eines Kristallkorns, ausgedrückt durch a/b, 1,2 oder weniger beträgt, bestimmt durch ein Messverfahren, wie es im Abschnitt "(B) Sn-Verhältnis" der Beschreibung beschrieben ist, wobei das Stahlmaterial durch ein Verfahren erhältlich ist, das die folgenden Schritte enthält:
einen Schritt der Herstellung einer Bramme mit einer chemischen Zusammensetzung, wie sie vorstehend in Bezug auf das Stahlmaterial angegeben ist,
einen Erwärmungsschritt des Erwärmens der Bramme auf eine Temperatur im Bereich von 1000 bis 1150°C,
einen Vorwalzschritt des Anwendens von Vorwalzen auf die Bramme,
einen Fertigwalzschritt des Anwendens von Fertigwalzen auf die Bramme, die dem Vorwalzen unterzogen wurde, um eine Walzendtemperatur der Oberfläche von 900 bis 750°C und eine Walzreduktionsrate ausgehend von 950°C von 50% oder mehr zu erzielen,
einen ersten beschleunigten Kühlungsschritt des Durchführens von beschleunigtem Kühlen des fertiggewalzten Stahlmaterials mit einer Kühlungsrate von 5 bis 10°C/s, bis die Oberflächentemperatur 630°C oder weniger erreicht,
einen Rekuperationsschritt des Unterbrechens der beschleunigten Kühlung des Stahlmaterials nach dem ersten beschleunigten Kühlungsschritt und des Kühlenlassens an der Luft für 30 bis 120 Sekunden und ferner die Rekuperation durch die Wärme aus dem Inneren des Stahlmaterials, bis die Oberflächentemperatur einen Bereich von 650 bis 700°C erreicht,
einen zweiten beschleunigten Kühlungsschritt des Durchführens von beschleunigtem Kühlen des Stahlmaterials nach dem Rekuperationsschritt mit einer Kühlungsrate von 10 bis 60°C/s, bis die Oberflächentemperatur 550°C oder weniger erreicht, und
einen Luftkühlungsschritt des Durchführens von Kühlung an der Luft nach dem zweiten beschleunigten Kühlungsschritt.

2. Das Stahlmaterial nach Anspruch 1 in Form von Stahlblech mit einer Blechdicke von 6 bis 100 mm.

3. Ein Verfahren zur Herstellung eines Stahlmaterials, wobei das Verfahren beinhaltet:
einen Schritt der Herstellung einer Bramme, bestehend aus, in Massenprozent:
von 0,01 bis 0,20% C,
von 0,01 bis 1,00% Si,
von 0,05 bis 3,00% Mn,
von 0 bis 0,050% P,
von 0 bis 0,0100% S,
von 0,05 bis 0,25% Sn,
von 0 bis 0,100% Al,
von 0,0005 bis 0,0100% N,
von 0,0001 bis 0,0100% O,
von 0 bis 0,050% Ti,
von 0 bis 0,050% Nb,
von 0 bis 0,050% V,
von 0 bis 0,050% W,
von 0 bis 0,050% Mo,
von 0 bis 0,10% Cu,
von 0 bis 0,05% Ni,
von 0 bis 0,10% Cr,
von 0 bis 0,05% Sb,
von 0 bis 0,0010% B,
von 0 bis 0,0100% Ca,
von 0 bis 0,0100% Mg,
von 0 bis 0,0100% Seltenerdmetallen und
einem Rest, der aus Fe und Verunreinigungen besteht,
einen Erwärmungsschritt des Erwärmens der Bramme auf eine Temperatur im Bereich von 1000 bis 1150°C,
einen Vorwalzschritt des Anwendens von Vorwalzen auf die Bramme,
einen Fertigwalzschritt des Anwendens von Fertigwalzen auf die Bramme, die dem Vorwalzen unterzogen wurde, um eine Endtemperatur der Oberfläche von 900 bis 750°C und eine Walzreduktionsrate ausgehend von 950°C von 50% oder mehr zu erzielen,
einen ersten beschleunigten Kühlungsschritt des Durchführens beschleunigter Kühlung des fertiggewalzten Stahlmaterials mit einer Kühlungsrate von 5 bis 10°C/s, bis die Oberflächentemperatur 630°C oder weniger erreicht,
einen Rekuperationsschritt des Unterbrechens der beschleunigten Kühlung des Stahlmaterials nach dem ersten beschleunigten Kühlungsschritt und des Kühlenlassens an der Luft für 30 bis 120 Sekunden und ferner die Rekuperation durch die Wärme aus dem Inneren des Stahlmaterials, bis die Oberflächentemperatur einen Bereich von 650 bis 700°C erreicht,
einen zweiten beschleunigten Kühlungsschritt des Durchführens von beschleunigtem Kühlen des Stahlmaterials nach dem Rekuperationsschritt mit einer Kühlungsrate von 10 bis 60°C/s, bis die Oberflächentemperatur 550°C oder weniger erreicht, und
einen Luftkühlungsschritt des Durchführens von Kühlung an der Luft nach dem zweiten beschleunigten Kühlungsschritt;
um ein Stahlmaterial mit einem Sn-Verhältnis einer Sn-Konzentration, a, in Atom%, an einer Kristallkorngrenze zu einer Sn-Konzentration, b, in Atom%, im Inneren eines Kristallkorns, ausgedrückt durch a/b, von 1,2 oder weniger, bestimmt durch ein Messverfahren, wie es im Abschnitt "(B) Sn-Verhältnis" der Beschreibung beschrieben ist, bereitzustellen.

4. Das Verfahren nach Anspruch 3, wobei das Stahlmaterial in Form von Stahlblech mit einer Blechdicke von 6 bis 100 mm vorliegt.

## Revendications

1. Matériau en acier, consistant, en termes de pourcentages en masse, en :
0,01 à 0,20 % de C,
0,01 à 1,00 % de Si,
0,05 à 3,00 % de Mn,
0 à 0,050 % de P,
0 à 0,0100% de S,
0,05 à 0,25 % de Sn,
0 à 0,100 % d'Al,
0,0005 à 0,0100 % de N,
0,0001 à 0,0100 % de O,
0 à 0,050 % de Ti,
0 à 0,050 % de Nb,
0 à 0,050 % de V,
0 à 0,050 % de W,
0 à 0,050 % de Mo,
0 à 0,10 % de Cu,
0 à 0,05 % de Ni,
0 à 0,10 % de Cr,
0 à 0,05 % de Sb,
0 à 0,0010% de B,
0 à 0,0100% de Ca,
0 à 0,0100 % de Mg,
0 à 0,0100 % d'éléments des terres rares (REM), et
le reste consistant en Fe et impuretés,
dans lequel le rapport du Sn de la concentration de Sn a, en % atomiques, à une limite de grain cristallin, à la concentration de Sn b, en % atomiques, à l'intérieur d'un grain cristallin, représenté par a/b, est de 1,2 ou moins, déterminé par une méthode de mesure telle que décrite dans la section "(B) rapport du Sn" de la description, lequel matériau en acier peut être obtenu par une méthode contenant les étapes suivantes :
une étape de préparation d'une brame ayant une composition chimique telle qu'indiquée ci-dessus à propos du matériau en acier,
une étape de chauffage dans laquelle la brame est chauffée à une température située dans la plage allant de 1000 à 1150 °C,
une étape de laminage grossier dans laquelle un laminage grossier est appliqué à la brame,
une étape de laminage de finition dans laquelle un laminage de finition est appliqué à la brame ayant subi le laminage grossier pour assurer une température de finition de la surface de 900 à 750 °C et un taux de réduction par laminage à partir de 950 °C de 50 % ou plus,
une première étape de refroidissement accéléré dans laquelle un refroidissement accéléré du matériau en acier ayant subi le laminage de finition est effectué à une vitesse de refroidissement de 5 à 10 °C/s jusqu'à ce que la température de la surface atteigne 630 °C ou moins,
une étape de récupération dans laquelle le refroidissement accéléré du matériau en acier est suspendu après la première étape de refroidissement accéléré, après quoi il est laissé à refroidir dans l'air pendant 30 à 120 secondes, et en outre la chaleur depuis l'intérieur du matériau en acier est laissée à être récupérée jusqu'à ce que la température de la surface devienne située dans la plage allant de 650 à 700 °C,
une deuxième étape de refroidissement accéléré dans laquelle un refroidissement accéléré du matériau en acier après l'étape de récupération est effectué à une vitesse de refroidissement de 10 à 60 °C jusqu'à ce que la température de la surface atteigne 550 °C ou moins, et
une étape de refroidissement par air dans laquelle un refroidissement dans l'air est effectué après la deuxième étape de refroidissement accéléré.

2. Matériau en acier selon la revendication 1 sous la forme d'une plaque en acier ayant une épaisseur de plaque de 6 à 100 mm.

3. Méthode de production d'un matériau en acier, laquelle méthode comprend :
une étape de préparation d'une brame consistant, en termes de pourcentages en masse, en :
0,01 à 0,20 % de C,
0,01 à 1,00 % de Si,
0,05 à 3,00 % de Mn,
0 à 0,050 % de P,
0 à 0,0100% de S,
0,05 à 0,25 % de Sn,
0 à 0,100 % d'Al,
0,0005 à 0,0100 % de N,
0,0001 à 0,0100 % de O,
0 à 0,050 % de Ti,
0 à 0,050 % de Nb,
0 à 0,050 % de V,
0 à 0,050 % de W,
0 à 0,050 % de Mo,
0 à 0,10 % de Cu,
0 à 0,05 % de Ni,
0 à 0,10 % de Cr,
0 à 0,05 % de Sb,
0 à 0,0010% de B,
0 à 0,0100 % de Ca,
0 à 0,0100 % de Mg,
0 à 0,0100 % d'éléments des terres rares (REM), et
le reste consistant en Fe et impuretés,
une étape de chauffage dans laquelle la brame est chauffée à une température située dans la plage allant de 1000 à 1150 °C,
une étape de laminage grossier dans laquelle un laminage grossier est appliqué à la brame,
une étape de laminage de finition dans laquelle un laminage de finition est appliqué à la brame ayant subi le laminage grossier pour assurer une température de finition de la surface de 900 à 750 °C et un taux de réduction par laminage à partir de 950 °C de 50 % ou plus,
une première étape de refroidissement accéléré dans laquelle un refroidissement accéléré du matériau en acier ayant subi le laminage de finition est effectué à une vitesse de refroidissement de 5 à 10 °C/s jusqu'à ce que la température de la surface atteigne 630 °C ou moins,
une étape de récupération dans laquelle le refroidissement accéléré du matériau en acier est suspendu après la première étape de refroidissement accéléré, après quoi il est laissé à refroidir dans l'air pendant 30 à 120 secondes, et en outre la chaleur depuis l'intérieur du matériau en acier est laissée à être récupérée jusqu'à ce que la température de la surface devienne située dans la plage allant de 650 à 700 °C,
une deuxième étape de refroidissement accéléré dans laquelle un refroidissement accéléré du matériau en acier après l'étape de récupération est effectué à une vitesse de refroidissement de 10 à 60 °C jusqu'à ce que la température de la surface atteigne 550 °C ou moins, et
une étape de refroidissement par air dans laquelle un refroidissement dans l'air est effectué après la deuxième étape de refroidissement accéléré ;
pour former un matériau en acier ayant un rapport du Sn de la concentration de Sn a, en % atomiques, à une limite de grain cristallin, à la concentration de Sn b, en % atomiques, à l'intérieur d'un grain cristallin, représenté par a/b, de 1,2 ou moins, déterminé par une méthode de mesure telle que décrite dans la section "(B) rapport du Sn" de la description.

4. Méthode selon la revendication 3, dans laquelle le matériau en acier est sous la forme d'une plaque en acier ayant une épaisseur de plaque de 6 à 100 mm.
